

Aug. 14, 1928.

1,680,667

A. M. CURTIS

ELECTROMAGNETIC DEVICE

Filed Oct. 3, 1922

2 Sheets-Sheet 1

Fig. 1.



Fig. 2.



Fig. 5.



Inventor:  
Austen M. Curtis  
by C. L. Sprague. Atty.

Aug. 14, 1928.

1,680,667

A. M. CURTIS

ELECTROMAGNETIC DEVICE

Filed Oct. 3, 1922

2 Sheets-Sheet 2

Fig. 3.



Fig. 4.



Inventor:  
Austen M. Curtis  
by C.G. Sprague Atty

## UNITED STATES PATENT OFFICE.

AUSTEN M. CURTIS, OF EAST ORANGE, NEW JERSEY, ASSIGNOR TO WESTERN ELECTRIC COMPANY, INCORPORATED, OF NEW YORK, N. Y., A CORPORATION OF NEW YORK.

## ELECTROMAGNETIC DEVICE.

Application filed October 3, 1922. Serial No. 592,028.

This invention relates to an electromagnetic device and in particular to a sensitive relay especially suitable for use in connection with high speed telegraph lines.

5 It is the principal object of the invention to provide a relay of high sensitivity and one in which the residual magnetism of the magnetic circuit is reduced to the lowest point possible.

10 A preferred embodiment of the invention is described and illustrated in the following specification and accompanying drawing in which Fig. 1 is a plan view. Fig. 2 is a side elevation of the relay shown in Fig. 1. Figs. 15 3 and 4 are typical wave forms illustrated to aid in explaining the operation of the relay under various service conditions, and Fig. 5 shows graphically the contact pressures obtained with such a relay for given operating currents and also the residual effect due to 20 various operating currents when employing different materials for the magnetic circuit.

Recent developments in the design of long submarine cables have increased the need for 25 a telegraph relay which is accurate and reliable when operated at high speeds with weak operating currents. According to this invention a very great improvement is obtained by the use of a new material for the 30 magnetic circuit. An investigation has shown that there have been obtained by the use of this material unexpected improvements in the operation of relays not only of the type particularly adapted for use with 35 submarine cables but of types suited for more general use.

In sending telegraph messages at high speed over long loaded telephone lines, as is 40 customary in composited systems, the presence of the loading coils makes it necessary to keep down the amplitude of the telegraph current impulses in order to prevent making the lines noisy by producing what is commonly called "Morse thump". Accordingly 45 on such lines a relay is required of much higher sensitivity than is required on unloaded lines where it is not necessary to limit the amplitude of the current impulses. Again, in the operation of long submarine 50 cables, the sending voltage is made as high as safety permits (60 volts being the safe limit for ordinary operation for long cables)

and with the sending voltage thus fixed, the speed of sending is limited to that which will permit the receiving of legible signals. 55

In telegraph systems employed on long submarine cables, particularly those designed to operate in connection with a printing telegraph receiver, it is very important to provide an accurate receiving relay which is constant in adjustment. In such systems the wave forms of the received signal currents differ quite materially from the wave forms of the ordinary land telegraph lines. In such a cable the high frequencies are attenuated to a much greater extent than the lower frequencies and as a result the wave forms of the current pulsations instead of being "square topped" are rounded to more nearly approach a sine wave form. With a square 70 top wave form the steepness of the wave front makes the point of operation of the relay quite certain, whereas with a rounded wave form the current wave does not for some time reach the necessary amplitude to 75 operate the relay and the time of operation therefore will depend more or less upon the slope of the wave. Since the time of operation of the relay is delayed somewhat it is desirable to provide a relay which will operate on currents of very small amplitude. 80

When operating with signal impulses having a rounded wave form, the time of operation is more uncertain, as explained below, and, moreover, the time of contact closure also is 85 less as a result of the comparatively slower movement of the armature. A square-topped wave having a steep front insures rapid acceleration of the armature and therefore a short period of armature travel, whereas 90 with a rounded wave form the acceleration of the armature is less rapid and the period of contact closure correspondingly decreased. The rounded wave form also produces the same uncertainty in the time of the release 95 of the relay and makes it desirable to provide a magnetic circuit in which the residual effect is as nearly negligible as possible. The uncertainty in the time of operation and time of release of a relay operating on a current 100 of rounded wave form, as well as the shorter period of contact closure, results in distorted signals, which are especially serious when using printing telegraph apparatus. If the

signal is received on a tape, as for example, by means of a siphon recorder, it is possible for the receiving operator to diligently study the tape and decipher the intended signal characters even though considerably distorted, but if a printing mechanism is employed a substantially undistorted signal is required in order that an intelligible message may be printed. Therefore in order to permit operation at high speed on such a cable, the requirements call for a relay which is sensitive and uniform both in operation and in release.

The unsatisfactory operation of a relay on currents having rounded wave forms may be overcome to a large degree by increasing the current strength in case circuit conditions permit such a procedure. However, if this is done and the material of the magnetic circuit is worked at a correspondingly higher flux density, the residual magnetism becomes greater and further increases the uncertainty of the point of operation of the relay.

In order to obtain efficient operation in cable circuits the use of the Gulstad vibrating circuit is often resorted to. When using the relay of this invention in this circuit, which is described in detail in the Electrical Review of London, volume 42, page 751, June 3, 1898, and volume 51, page 247, August 22, 1902, only sufficient current need be supplied over the line to control the action of a pair of windings since the circuit contemplates the use of local batteries to furnish the operating current for the relay. By the use of this circuit the operation of the relay is materially improved, especially in cable service. Not only does the relay operate on smaller line currents, but also there is much less distortion of the signals. However, with this circuit it is necessary to maintain the magnetic circuit of the relay highly balanced, since after the balance is upset the armature becomes biased, thus destroying the "trigger action" of the circuit and impairing the operation of the relay. Such magnetic biases are likely to occur when the relay receives an abnormal value of current and the portion of the resulting flux which remains upsets the balanced action of the polarizing flux in the armature of the relay. In accordance with this invention there is brought about a decrease in the residual magnetization of the relay employed in the Gulstad circuit resulting in an increased efficiency in the operation of the relay.

In the relay which is illustrated in Figs. 1 and 2, there is provided a mounting plate 6 of non-magnetic material having lugs 7, 7, to which are secured the L-shaped pole pieces 8 and 9. The armature 10 is rigidly clamped between the rear ends of the pole pieces by means of screws 11, 11, thin non-magnetic shims 12, 12 being inserted as

shown to provide a pair of fixed gaps in the magnet circuit. The armature 10 which extends through a hollow spool 13 upon which are wound the operating windings, is free to vibrate as a beam in a plane parallel to the base of the relay, its free end being in operating relation with the adjusting screws 14, 15, which are provided with fine threads and threaded into the ends of pole pieces 8 and 9 respectively. In order to preclude the possibility of the armature coming in direct contact with the adjusting screws, stop-pins 5-5 of brass or other non-magnetic material are secured to the armature as shown. Attached to the free end of armature 10 are the contact springs 16, 16, the other ends of which are adapted, upon movement of the armature, to engage contact screws 17, 17 supported upon suitable brackets 18, 18 which are insulated from the mounted plates by means of suitable insulating members 20, 20. The free ends of springs 16, 16 are adapted to be in sliding engagement with each other in order to overcome any tendency to chatter when the springs make contact with the contact screws. A U-shaped permanent magnet 21 is mounted on the lower side of mounting plate 6 and is joined in magnetic circuit with the pole pieces 8 and 9 by the magnetic members 22 and 23. The gaps at the rear of the magnetic circuit are equal and fixed, while the working air gaps at the front of the magnetic circuit may be very accurately adjusted by turning the adjusting screws 14, 15 which are provided with fine threads. In the operation of the relay, the armature is deflected or bent under the influence of the forces set up in the front magnetic air gaps by the polarizing and operating fluxes thus making and breaking contact with the contact screws 17, 17. The strength of the permanent magnet 21 is such that the pull exerted thereby upon the armature 10 is practically sufficient to counteract the stiffness of the armature which is therefore substantially in equilibrium.

The permanent magnet is preferably made from tungsten steel and the path of the polarizing flux through the magnetic circuit is from one limb of the permanent magnet through the contact block 22 to the front end of pole piece 8. Here the flux divides into two paths, one is back through the pole piece, across the two non-magnetic shims 12, 12 and the clamped end of armature 9 into pole piece 9 and thence to the other limb of the permanent magnet, through block 23. The other path is into the adjusting screw 14 across the working air gaps and the free end of armature 10 to adjusting screw 15 thence into pole piece 9 and returning to the other limb of permanent magnet through contact block 23. It will be seen that both the amount and the direction of the polarizing

flux through the armature depends upon the position of the free end of the armature and the working air gaps. When the armature is exactly midway between the adjusting screws, there is no polarizing flux through the armature in the direction of its length since it connects two points of equal magnetic potential, but as it moves toward one adjusting screw, the polarizing flux flows through the armature in a positive direction, whereas when it moves toward the opposite adjusting screw, the polarizing flux reverses and flows through the armature in a negative direction.

15 The paths of the operating flux, or that flux which is generated by currents traversing the operating windings, is out from the front end of armature 10 across the two working air gaps in parallel into the adjusting screws 14, 15, through the non-magnetic shims 12, 12 to the rear end of the armature. There is a third path for this operating flux through the permanent magnet, but due to the high reluctance of the permanent magnet as compared to that of the pole pieces, practically none of the flux returns by this path. It will be seen from the above that this relay differs from most all other types of polarized relays in that when the relay operates to deflect the armature from one side to the other, both the operating flux and the polarizing flux reverse through the armature which accounts for the fact that the relay is highly sensitive to the magnetic characteristics of the armature. When employing silicon steel as the material for the armature 10 and a high grade of magnetic iron for the pole pieces 8 and 9 and the contact blocks 22 and 23 the relay operates on a very small current, but when operating at high speed, the residual effect of the magnetic circuit slows down the operation and causes distortion. This residual effect was first somewhat decreased by restricting the cross section of a portion of the armature, as shown at 25, but the operation of the relay both as regards sensitivity and speed were still limited by the remaining residual effect. In fact it has been determined by careful tests that this remaining residual magnetism increases the minimum operating current approximately 8.7 times.

In Figs. 3 and 4 are shown typical wave forms representing respectively a square-topped signal impulse usual in land telegraphy and a rounded top signal impulse as present in long submarine cable systems. The time scale for these curves is about fifty cycles per second, thus giving a single impulse in about one hundredth of a second. The position of the armature in relation to the contact members is shown by the lower curve in each of Figs. 3 and 4. At 25 the armature breaks contact at one side and 65 swings across, and at 26 makes contact with

the other side. It is inevitable that, due to temperature and other conditions, there will be more or less uncertainty in the value of current at which the armature of the relay starts to move. Should it be assumed, for example, that in Figs. 3 and 4 operation will occur at current values between points 27 and 28, this latter being twice the value of the former, this means that the operation will be determined within a range of time of less than half a thousandth of a second for Fig. 3 with its square-topped wave, whereas the time range of uncertainty is nearly two thousandths of a second for Fig. 4. This comparison shows how the uncertainty as to the exact current values for operation gives much greater uncertainty for the time of operation for the rounded top wave of Fig. 4 than for the square-topped wave of Fig. 3.

Another respect in which Fig. 4 shows at a disadvantage compared to Fig. 3 is that the time of travel of the relay armature will be longer for Fig. 4 than for Fig. 3. In Fig. 3 let it be assumed that the armature resting on one contact moves away from that contact at 27. Some time will elapse for the armature to travel across from the position indicated at 25 to that indicated at 26, but within less than half a thousandth of a second the current will have risen to double the value at which the break occurred, that is, from 27 to 28. This rapid increase of current produces a strong acceleration of the armature and causes it to move quickly, as shown at 25 and 26. However, in Fig. 4 the elapsed time for the current to double in value is nearly two thousandths of a second so that the travel of the armature will consume a longer time, as indicated from 25' to 26'. It will be seen that the contact closure on one side for Fig. 3 from 26 to 29 is about twice as long as on the other side from 30 to 31, but in Fig. 4 the corresponding closure from 26' to 29' is nearly three times as long as from 30' to 31'. Moreover, this distortion of signals would be increased by the uncertainty as to the point of operation of the relay. Thus, if the contact broke at 33 instead of 32, the resulting signal received would be shortened to the time represented by 30''-31' which is less than a third as long as from 26' to 29' whereas the signal should be half as long.

There is still another respect in which the disadvantage of the wave shape of Fig. 4 becomes manifest compared with Fig. 3. The flexibility of the spring contact members 16 permits the end of the armature 25 to continue its movement a little further toward the adjusting screws 15 after the contact is made. The end of the armature 25 then springs back a little, but if the current in the coil 13 is strong enough, the contact is not broken. Such oscillations at the

end of the armature 25 may continue through several periods, but if a strong current is maintained in the coil 13, the contact will not be broken and there will be no 5 chattering. This will be the manner of operation for Fig. 3. It will be seen that after the contact is made at the time indicated by the point 26, a strong holding current is maintained for as much as seven or eight 10 thousandths of a second. During this time the oscillation of the armature is damped out by the type of contact springs employed. However, in Fig. 4 it will be seen that when the contact is made at 26', the current is 15 already beginning to die down and a fluttering of the end of the armature may continue until the current becomes so weak that it will not hold the contact closed, thus making it possible for a certain amount of chattering, as at the point 35. If the dotted lines 20 of armature travel 29" to 30" be assumed, it will be seen that closure is not effected until after the peak current is passed and the tendency for the armature flutter to develop into contact chattering will be even 25 more probable.

Since in long submarine cable systems the received current impulses are of the rounded wave form, it is essential that a relay for 30 use in such systems be capable of satisfactory operation on current impulses of that form. It therefore follows that the magnetic circuit of the relay must not only be very sensitive for operation, but must eliminate so far as possible the effect of residual 35 magnetism which makes the operation of the relay uncertain.

The requirement of high sensitivity is particularly urgent in connection with a relay 40 operated at high speeds since under such conditions it is necessary to insure rapid travel of the armature, in order to obtain satisfactory closure of contacts and only with a relay of high sensitivity is it possible 45 to obtain sufficiently rapid travel with the small currents available.

Although at first glance it might seem that the residual effect of such a relay is due principally to the remanence of the material 50 used, such is not the case, due to the numerous gaps in the magnetic circuit and the resulting demagnetizing effect of the poles at such gaps, but is due chiefly to the coercive force or coercivity of the material 55 of which the magnetic circuit is composed.

Silicon steel which has been largely used in relays heretofore not only is objectionable because of its comparative brittleness and the difficulty of working it, but also because 60 it has a comparatively high coercive force. A magnetic material known as permalloy when given a suitable heat treatment has been found to have a permeability at low magnetizing force greater than that 65 of iron and a coercivity much below that of

iron. This material is described and claimed in patent to G. W. Elmen 1,586,884 issued June 1, 1926. Particularly good results were obtained in tests when employing a variety of permalloy prepared by fusing nickel and 70 iron together in the proportion of 78½ per cent nickel and 21½ per cent iron, good commercial grades of these materials being suitable for this purpose. Good results may be obtained when the nickel content predominates and the rest is iron or iron with small 75 per cents of other elements which may be present as impurities or to increase the resistivity, as may be done for example by adding chromium. The fused composition is poured into a mold to bring it at once to the proper shape, or it may be brought to the desired shape after molding by being hammered, swaged, drawn, rolled, or worked in any other simple manner. After being 80 brought to the desired shape, the composition is given a heat-treatment to develop therein the highest permeability possible at low magnetizing forces and the lowest possible coercive force. According to present 85 practice, this is done by heating the desired shapes to a temperature of about 850° C., maintaining it at that temperature for a few minutes to insure a uniform temperature throughout, then cooling slowly to a temperature of about 600° C. which is just about the critical or transition temperature of the 90 alloy, that is, the temperature at which the magnetic properties disappear on heating and reappear on cooling; and finally cooling 95 from that temperature more rapidly but at a definite rate dependent upon the ratio of nickel to iron in the alloy. A convenient 100 method of securing the desired rate of cooling after the material has been maintained for a few minutes at a temperature of 850° C. has been found to be a rapid withdrawing 105 of the material from the furnace and placing it in a blast of air which is controlled to secure a desired rate of cooling. The necessary 110 cooling will always be at a rate intermediate that required for annealing and that at which such strains would be set up in the material as to lower its permeability below the desired value. The results of tests on a 115 relay of the type described in which the magnetic circuit is composed of this variety of permalloy as compared with the results of an exactly identical relay in which the armature is made from silicon steel and the 120 pole pieces from a high grade of magnetic iron are shown on Fig. 5 of the drawing.

Curve A shows the contact pressures obtainable for various operating currents with a relay having a magnetic circuit of high grade magnetic iron except for the armature which is of silicon steel. Curve B shows the contact pressures obtainable under the same conditions with a relay having a magnetic circuit of permalloy but otherwise

identical with the relay of curve A in construction and adjustment. Curve A' shows the residual effect or the contact pressure of the relay of curve A, immediately after the 5 various operating currents had been removed. Curve B' shows the residual contact pressures for the relay of curve B in which the magnetic circuit is of permalloy. The contact pressures shown in curves A' 10 and B' are due chiefly to the coercive forces of the materials used in the magnetic circuits although these pressures are, to a very slight degree, augmented as a result of the flux from the permanent magnet due to the 15 armature being in its deflected position. The minimum direct current operating value of the relay employing a silicon steel armature and magnetic iron pole pieces was .060 milliamperes as compared to a similar minimum 20 operating current for the nickel iron alloy of .032 milliamperes. For current values of the order of the minimum operating current, the relay having the nickel iron alloy magnetic circuit operates with a much higher 25 contact pressure and therefore is more satisfactory and has less tendency to chatter. Although for operating currents above one millampere the contact pressure of the relay having the permalloy magnetic circuit is less, 30 we are chiefly concerned with the contact pressures at the minimum operating currents and for this reason the relay having the permalloy magnetic circuit is far superior.

In order to assure that this relay will operate satisfactorily under service conditions, it 35 is necessary to determine the residual magnetism in the relay after operation with a maximum current which may be as high as 15 milliamperes. Referring to the curve, it 40 will be noted that with the relay having the silicon steel armature, the residual effect after being operated on a current of 15 milliamperes is approximately  $4\frac{1}{4}$  grams whereas the residual pull under the same conditions 45 for the permalloy relay is less than  $\frac{1}{2}$  gram. By thus reducing the residual effect, the operation of the relay is improved very materially and distortion of signals is overcome to a large extent.

50 In addition to the advantage accruing from higher permeability at low magnetizing forces and a lower coercive force, the relay with permalloy is also quicker acting due to the low hysteresis loss of the material. 55 The comparatively high hysteresis loss in an armature employing a material, such as magnetic iron or silicon steel, produces power losses which oppose the motion of the armature by reducing the flux density caused by 60 a varying current, whereas in a relay employing an armature of permalloy the movement of the armature is less sluggish due to its low hysteresis loss and the relay therefore operates more satisfactorily on high 65 speed telegraph systems.

Since, as already referred to, both the polarizing and operating fluxes reverse in the armature when the relay operates, the magnetic characteristics of the armature are of great importance. When using permalloy 70 for the armature and a high grade of magnetic iron for the other portions of the magnetic circuit the operation shows a decided improvement over that of a similar relay having a silicon steel armature although as would be expected, the improvement is not as great as when the entire magnetic circuit is composed of the nickel iron 75 alloy.

By the term "low magnetizing force" is 80 meant a force of a few tenths of a gauss.

A particular type of sensitive relay having the improved magnetic circuit of this invention has been described above, but the invention in its broader aspects is not limited to any one type or form of relay being applicable wherever one or more of the advantages mentioned can be obtained.

What is claimed is:

1. An electromagnet device comprising an 90 energizing coil, pole pieces therefor, an armature and a magnetic circuit including said armature and pole pieces composed of a material comprising nickel and iron of such low coercivity that the armature operates at a precise current value substantially 95 independent of its previous magnetic condition.

2. An electromagnet device comprising an 100 energizing coil, pole pieces therefor, an armature and a magnetic circuit including 105 said armature and pole pieces having a portion thereof composed of a nickel-iron alloy of such low coercivity that the armature operates at a precise current value substantially independent of its previous magnetic condition.

3. An electromagnetic device comprising an energizing coil, pole pieces therefor, an 110 armature, and a magnetic circuit including said armature and pole pieces having a portion thereof composed of a nickel-iron alloy of such low coercivity that the armature is released at a precise current value substantially 115 independent of the operating current value.

4. A relay to operate with precision of response at a definite input current consisting of an input winding, pole pieces therefor, relay contacts, and an armature controlling said contacts and actuated by flux developed in said pole pieces, the magnetic circuit comprising said core and armature having at least a considerable portion thereof composed of a nickel iron alloy with substantially lower coercivity than iron, whereby the armature operates at a precise current value substantially independent of the earlier magnetic condition of said core.

5. An electromagnetic device comprising 130

an energizing coil, pole pieces therefor, means for polarizing said pole pieces, a balanced magnetic circuit including said armature so arranged that both the polarizing flux and the flux produced by the energizing coil are reversed in direction with movement of the armature, said armature being composed of a nickel iron alloy of such low coercivity that the armature is operated at 10 a precise current value substantially independently of its earlier magnetic condition.

6. An electromagnetic relay comprising an energizing coil, pole pieces therefor, an armature and a magnetic circuit including 15 said pole pieces and armature, composed of a material containing at least two members of the magnetic group of metals and having such low coercivity that the contact pressure

exerted by said armature due to residual magnetism is less than one fifth that under 20 the same operating conditions in a similar relay having a silicon steel armature and pole pieces.

7. A polar relay designed to operate on current received over a high speed, long, 25 loaded submarine telegraph cable comprising an armature, a coil for actuating said armature, and pole pieces completing a magnetic circuit through said armature, said armature and pole pieces being composed 30 of a nickel iron alloy having a coercivity less than .06.

In witness whereof, I hereunto subscribe my name this 30th day of September, A. D. 1922.

AUSTEN M. CURTIS.